# EUROPEAN PATENT SPECIFICATION

(11) **EP 1 474 566 B1**
(45) Date of publication and mention of the grant of the patent: **26.07.2006**
(21) Application number: 02792969.4
(22) Date of filing: 03.12.2002
(51) Int. Cl.: D07B 1/06

(54) **COMPACT STEEL CORD**
KOMPAKTES STAHLSEIL
CABLE D'ACIER COMPACT

(30) Priority: 14.02.2002 EP 02100137
(43) Date of publication of application: 10.11.2004
(73) Proprietor: N.V. BEKAERT S.A., 8550 Zwevegem (BE)
(72) Inventor: MEERSSCHAUT, Dirk, B-8710 Ooigem (BE); PILLE, Johan, B-8800 Roeselare (BE); VANNESTE, Stijn, B-8770 Ingelmunster (BE)
(86) International application number: PCT/EP2002/014077
(87) International publication number: WO 2003/069055

(56) References cited:
- EP-A- 0 675 223
- EP-B- 0 627 520
- WO-A-01/49926

## Description

### Field of the invention.

The present invention relates to a steel cord adapted for the reinforcement of elastomer products. The steel cord comprises a core filament with a core filament diameter and layer filaments twisted around the core filament in the same direction and with the same step.

### Background of the invention.

Steel cords where all the steel filaments are twisted in the same direction and with the same step are known in the art and are often referred to as "compact steel cords" since they may lead to a compact cross-sectional configuration with a high amount of steel within a limited cross-sectional surface area.
Within the group of compact steel cords, following configurations are widely used in the art of elastomer reinforcement:
- 3xd_{c} |9xd_{*l*} CC
- 1xd_{c} | 18xd_{*l*} CC
A 3xd_{c}| 9d_{*l*} CC is a compact cord comprising three core filaments with a core filament diameter d_{c} and nine layer filaments with a layer filament diameter d_{*l*}. The core filament diameter d_{c} is somewhat greater than the layer filament d_{*l*}. Such a compact cord is disclosed in US-A-4,788,815. A 1xd_{c} | 18xd_{*l*} CC is a compact cord comprising one core filament with a core filament diameter d_{c} and eighteen layer filaments with a layer filament diameter d_{*l*}, arranged in an intermediate layer of six filaments and an outer layer of twelve filaments. Such a compact cord is disclosed in EP-B1-0 627 520. Document WO 01/49926 A discloses a further multi-layer cable.
Both compact cords constitute stable constructions and may be used to reinforce the carcass plies of medium to heavy truck and bus radial tires. A 1 xd_{c} | 18xd_{*l*} CC construction with its nineteen filaments is used for the higher breaking loads and a 3xd_{c}| 9xd_{*l*} CC construction with its twelve filaments is used for the lower breaking loads. The required breaking load is then met by a suitable choice of the filament diameters d_{c} and d_{*l*}.

By varying the diameters it is technically possible to cover such a broad range of breaking loads so that the carcass plies of practically all current medium and heavy truck and bus radial tires can be reinforced.
Although such a broad range is technically possible, it is, however, not always technically desirable. Increasing the filament diameters in order to obtain higher breaking loads results in decreasing values of fatigue resistance. So the filament diameter range has an upper limit due to technical reasons.
Decreasing the filament diameters in order to obtain lower breaking loads is technically desirable since it results in increasing values of fatigue resistance. Decreasing the filament diameters, however, has also its limits, since further drawing of the high carbon steel filaments is expensive. So the filament diameter range has a lower limit due to economical reasons.
Bearing in mind the lower and the upper limit, it is difficult, if not impossible with the two constructions 3xd_{c}| 9xd_{*l*} CC and 1xd_{c} | 18xd_{*l*} CC to cover the whole range of medium and heavy truck tires with technically and economically feasible steel cords.

### Summary of the invention.

It is an object of the present invention to fill in the gap between the two constructions 3xd_{c} | 9xd_{*l*} CC and 1xd_{c}| 18xd_{*l*} CC.
It is another object of the present invention to provide for a stable steel cord construction with an acceptable level of fatigue resistance.
It is a further object of the present invention to provide for a steel cord with a good fretting behavior.

According to the present invention there is provided a steel cord adapted for the reinforcement of elastomer products. The steel cord comprises a core filament with a core filament diameter d_{c} and 3N layer filaments twisted around said core filament in the same direction and with the same step. N ranges from four to five. The 3N layer filaments are arranged in an intermediate layer of N intermediate layer filaments and in an outer layer of 2N outer layer filaments. The layer filaments in the intermediate layer have an intermediate layer diameter d_{*i*}. The core filament diameter d_{c} is smaller than the intermediate layer diameter d_{*i*}. This invention cord is a compact cord. The cord has a good fretting behavior, a high breaking load per unit of cross-section and a small diameter. The cord has a symmetric stable construction. It has thirteen to sixteen filaments and fills in the gap between the 3×d_{c}| 9×d_{*l*} CC and 1 xd_{c} |18×d_{*l*} CC constructions.
The steel cord is adapted for the reinforcement of elastomer products, which means that it has a steel composition along the following lines : a minimum carbon content of 0.60 % (e.g. at least 0.80 %, or at least 0.92 % with a maximum of 1.2 %), a manganese content ranging from 0.20 to 0.90 % and a silicon content ranging from 0.10 to 0.90 % ; the sulphur and phosphorous contents are each preferably kept below 0.03 % ; additional elements such as chromium (up to 0.2 à 0.4 %), boron, copper, cobalt, nickel, vanadium ... may be added to the composition in order to minimize the amount of deformation needed to obtain a predetermined tensile strength. The steel filaments are generally covered with a coating layer to increase the resistance against corrosion or to enhance the adhesion with rubber. This coating may be a chemical primer or may be a metallic coating. The exact type of coating depends upon the eventual application. Corrosion resistant coatings are zinc or a zinc aluminum alloy. Adhesion coatings are brass in the case of rubber, or a so-called ternary brass such as copper-zinc-nickel (e.g. 64% / 35.5% / 0.5%) and copper-zinc-cobalt (e.g. 64% / 35.7% / 0.3%), or a copper-free adhesion layer such as zinc-cobalt or zinc-nickel. The final diameters of the steel filaments range from 0.05 mm to 0.60 mm. In case of reinforcement of carcass plies of tires, the filament diameters preferably range from 0.05 mm to 0.35 mm.

N is preferably equal to five, which means that the steel cord comprises sixteen filaments. Five is preferred to four since five filaments in the intermediate layer fill more the intermediate layer in a stable way.

Preferably the core filament diameter d_{c} is greater than the diameter of a circle tangent to each of the cross-sections of the intermediate layer filaments in the hollow space that remains free when their cross-sections have the highest packing density.

In a first preferable embodiment of the invention all 3N layer filaments, i.e. all N intermediate layer filaments and all 2N outer layer filaments have a same intermediate layer filament diameter d_{*i*}. This first preferable embodiment may be summarized by following formula : $1 {xd}_{c} | 3 {Nxd}_{i} CC$ This first embodiment has the advantage that only two different filament diameters are required.

In a second preferable embodiment of the invention the outer layer of 2N filaments has N filaments facing two intermediate layer filaments with a diameter equal to the intermediate layer diameter d_{*i*} and has N filaments facing only one intermediate layer filament with a diameter smaller than the intermediate layer diameter d_{*i*}.
This second embodiment has the advantage of a so-called Warrington construction with a round cross-section.

### Brief description of the drawings.

The invention will now be described into more detail with reference to the accompanying drawings wherein
- FIGURE 1 is a cross-section of a first embodiment of a steel cord according to the invention ;
- FIGURE 2 is an explanatory drawing ;
- FIGURE 3 is a cross-section of a second embodiment of a steel cord according to the invention.

### Description of the preferred embodiments of the invention.

FIGURE 1 shows a cross-section of a first embodiment of a steel cord 10. The steel cord comprises a core filament 12 with a core filament diameter d_{c}. Five intermediate layer filaments 14 form an intermediate layer around core filament 12. The intermediate layer filaments have a diameter d_{*i*}. Ten outer layer filaments 16 form an outer layer around the intermediate layer. The outer layer filaments 16 also have the same intermediate layer filament diameter d_{*i*}. All intermediate layer filaments 14 and all outer layer filaments 16 are twisted in the same twisting direction and with the same twisting step so that a compact configuration is formed. The cross-section has the typical form of a pentagon.

The core filament diameter d_{c} is smaller than the intermediate layer filament diameter d_{*i*}.
Referring to FIGURE 2, the core filament diameter d_{c} is greater than the diameter of a circle 15 tangent to each of the cross-sections of the intermediate layer filaments 16 in the hollow space that remains free when their cross-sections have the highest packing density.
A suitable example of a cord according to the first embodiment of the invention is :

| | |
|---|---|
| 1x0.14 \| 15x0.175 CC | twisting step = 11 mm |
| | twisting direction = S |

Other examples are :
1x0.175 | 15x0.22 CC
1x0.16 | 15x0.20 CC
1x0.13 | 15x0.16 CC
1x0.10 | 15x0.13 CC

FIGURE 3 shows a cross-section of a second embodiment of the steel cord 20 according to the invention. The steel cord 20 comprises a core filament 22. Five intermediate layer filaments 24 with an intermediate layer filament d_{*i*} have been twisted around the core filament 22. An outer layer of outer layer filaments 26, 28 is formed around the intermediate layer. Of the outer layer filaments 26, 28, those five outer layer filaments 26 facing two intermediate layer filaments 24 have a diameter equal to said intermediate layer diameter d_{*i*}. Five outer layer filaments 28 facing only one intermediate layer filament 24 have a diameter smaller than the intermediate layer diameter d_{*i*}.
In contrast with FIGURE 1, the cross-section has a round form.

Depending upon the steel composition used and upon the degree of final drawing, the steel cord can be carried out in various tensile versions, ranging from a normal tensile strength to an ultra high tensile strength.

The steel cords according to the invention can be manufactured by means of a tubular twisting machine or preferably by means of a double-twisting device.

Both embodiments may be provided or not with a wrapping filament wrapped around the other filaments. However, for use in carcass plies, the non wrapped version is preferred. In this non wrapped version, non sleeving of the steel cord may be obtained by suitably preforming the outer layer steel filaments so that the outer layer filaments exert a force which is directed radially inward. Such a preforming is disclosed in EP-B1-0 627 520.

Table 1 hereunder summarizes some properties measured on steel cords according to the first embodiment of the present invention.

**Table 1**

| **0.14\|15 x 0.175 CC** | | | |
|---|---|---|---|
| | Dimensions | High tensile strength | Super tensile strength |
| Twisting step | Mm | 11,4 | 11,6 |
| PLE | % | 0.083 | 0.080 |
| Diameter cord | mm | 0,834 | 0,840 |

| Tensile test not embedded | | | |
|---|---|---|---|
| Weight per length | g/m | 2,984 | 3,019 |
| Breaking load | N | 1238 | 1307 |
| Tensile strength | MPa | 3261 | 3404 |
| E-modulus | MPa | 189986 | 190397 |
| Total elongation at fracture | % | 2,44 | 2,36 |

| Tensile test embedded | | | |
|---|---|---|---|
| Breaking load | N | 1346,7 | 1415,7 |
| Tensile strength | MPa | 3547 | 3686 |
| E-modulus | MPa | 198183 | 197668 |
| Total elongation at fracture | % | 2,1 | 2,16 |

| Three point bending test not embedded | | | |
|---|---|---|---|
| εₖ = Eₖ | MPa | 152 | 160 |
| εᵥ = Eᵥ | MPa | 513 | 329 |
| Knee value Mᵥ | Nmm | 0,4 | 0,4 |
| A | % | 19 | 21 |

| Three point bending test embedded | | | |
|---|---|---|---|
| εₖ = Eₖ | MPa | 313 | 306 |
| εᵥ = Eᵥ | MPa | 855 | 810 |
| Knee value Mᵥ | Nmm | 3,6 | 3,8 |
| A | % | 31 | 35 |

| Compression test | | | |
|---|---|---|---|
| σₖ = Rₖ | M Pa | 172 | 257 |
| Wₖ | % | 0,88 | 1,28 |
| E compression modulus | MPa | 6066 | 7316 |

| Taber stiffness test Not embedded | | | |
|---|---|---|---|
| Mₒ | TSU | 27,6 | 31 |
| Mₒ' | TSU | 1,9 | 1,5 |
| Eₖ | MPa | 171 | 196 |
| V | % | 93 | 95 |

| Taber stiffness test Embedded | | | |
|---|---|---|---|
| Mₒ | TSU | 14,5 | 13,2 |
| Mₒ' | TSU | 1,5 | 1,2 |
| Eₖ | MPa | 431 | 398 |
| V | % | 90 | 91 |

| Three Roller Fatigue test | | | |
|---|---|---|---|
| Number of cycli before fracture | | 20006 | 30166 |

PLE or part load elongation expresses the elongation at very small loads below 50 Newton.

Information about the Taber stiffness test, the three point bending test, and the compression test can be read from L. BOURGOIS, Survey of Mechanical Properties of Steel Cord and Related Test Methods, Special Technical Publication 694, ASTM, 1980.

## Claims

1. A steel cord (10) adapted for the reinforcement of elastomer products, said steel cord comprising a core filament (12) with a core filament diameter and 3N layer filaments (14, 16) twisted around said core filament in the same direction and with the same step, N ranging from four to five, said 3N layer filaments being arranged in an intermediate layer (14) of N filaments and in an outer layer (16) of 2N filaments, the layer filaments in said intermediate layer having an intermediate layer diameter, wherein said core filament diameter is smaller than said intermediate layer diameter.

2. A steel cord (10) according to claim 1, wherein N equals five.

3. A steel cord (10) according to any one of the preceding claims, wherein said core filament (12) diameter is greater than the diameter of a circle tangent to each of the cross-sections of the intermediate layer filaments in the hollow space that remains free when their cross-sections have the highest packing density.

4. A steel cord (10) according to any one of the preceding claims, wherein all 3N layer filaments have said same intermediate layer diameter.

5. A steel cord (20) ccording to any one of claims 1 to 3, wherein said outer layer of 2N filaments has N filaments facing two intermediate layer filaments and having a diameter equal to said intermediate layer diameter and N filaments facing only one intermediate layer filament and having a diameter smaller than said intermediate layer diameter.

## Patentansprüche

1. Stahlseil (10), das zur Verstärkung von Elastomerprodukten geeignet ist, wobei das Stahlseil ein Kernfilament (12) mit einem Kernfilamentdurchmesser und 3N Schichtfilamente (14, 16) aufweist, die in derselben Richtung und mit demselben Schritt um das Kernfilament herum gewunden sind, wobei N im Bereich von vier bis fünf liegt, wobei die 3N Schichtfilamente in einer Zwischenschicht (14) aus N Filamenten und in einer äußeren Schicht (16) aus 2N Filamenten angeordnet sind, wobei die Schichtfilamente in der Zwischenschicht einen Zwischenschichtdurchmesser aufweisen, wobei der Kernfilamentdurchmesser kleiner ist als der Zwischenschichtdurchmesser.

2. Stahlseil (10) nach Anspruch 1, wobei N gleich fünf ist.

3. Stahlseil (10) nach einem der vorangehenden Ansprüche, wobei der Durchmesser des Kernfilaments (12) größer ist als der Durchmesser einer Kreistangente zu jedem der Querschnitte der Zwischenschichtfilamente in dem Hohlraum, der frei bleibt, wenn ihre Querschnitte die höchste Packungsdichte haben.

4. Stahlseil (10) nach einem der vorangehenden Ansprüche, wobei alle 3N Schichtfilamente den gleichen Zwischenschichtdurchmesser aufweisen.

5. Stahlseil (20) nach einem der Ansprüche 1 bis 3, wobei die äußere Schicht aus 2N Filamenten N Filamente aufweist, die zu zwei Zwischenschichtfilamenten weisen und einen Durchmesser haben, der gleich dem Zwischenschichtdurchmesser ist, und N Filamente aufweist, die nur zu einem einzigen Zwischenschichtfilament weisen und einen Durchmesser haben, der kleiner ist als der Zwischenschichtdurchmesser.

## Revendications

1. Câble d'acier (10) adapté pour renforcer des produits élastomères, ledit câble d'acier comprenant un filament d'âme (12) présentant un certain diamètre de filament d'âme et 3N filaments de couches (14, 16) torsadés autour dudit filament d'âme dans la même direction et avec le même pas, N étant compris entre quatre et cinq, lesdits 3N filaments de couche étant arrangés en une couche intermédiaire (14) de N filaments et une couche extérieure (16) de 2N filaments, les filaments de couche dans ladite couche intermédiaire présentant un certain diamètre de couche intermédiaire, dans lequel le diamètre dudit filament d'âme est plus petit que le diamètre de ladite couche intermédiaire.

2. Câble d'acier (10) selon la revendication 1, dans lequel N est égal à cinq.

3. Câble d'acier (10) selon l'une quelconque des revendications précédentes, dans lequel le diamètre dudit filament d'âme (12) est plus grand que le diamètre d'un cercle tangent à chacune des sections transversales des filaments de la couche intermédiaire dans l'espace creux qui reste libre lorsque leurs sections transversales présentent la densité de serrage la plus élevée.

4. Câble d'acier (10) selon l'une quelconque des revendications précédentes, dans lequel tous les 3N filaments de couche présentent le même diamètre de couche intermédiaire.

5. Câble d'acier (20) selon l'une quelconque des revendications 1 à 3, dans lequel ladite couche extérieure de 2N filaments comprend N filaments faisant face à deux filaments de couche intermédiaire et dont le diamètre est égal audit diamètre de couche intermédiaire, et N filaments faisant face à un seul filament de couche intermédiaire et dont le diamètre est plus petit que ledit diamètre de couche intermédiaire.
